

1

3,154,414  
IMAGE REMOVAL  
Vsevolod Tulagin, St. Paul, George H. Kolb, West St. Paul, and Donald K. Meyer, St. Paul, Minn., assignors to Minnesota Mining and Manufacturing Company, St. Paul, Minn., a corporation of Delaware  
No Drawing. Filed Apr. 18, 1960, Ser. No. 22,670  
6 Claims. (Cl. 96—1)

This invention relates to a new and useful method for removing latent images from photoconductive sheet materials and restoring them to a dark adapted state.

Successive production of latent images on a photoconductive sheet material is necessary in the preparation of colored reproductions by electrolytic deposition of colored materials on the photoconductor sheet material.

It is an object of this invention to make possible the preparation of a plurality of successive images on a photoconductive material in a simple, relatively fast, and convenient manner.

In the production of the images on a photoconductive sheet material, the photoconductive material is selectively exposed to a light source of the visible spectrum so that certain areas are rendered conductive after exposure. This retained conductivity makes possible the subsequent production of the images by electrolytic means. Where two or more successive images are to be applied the photoconductive sheet material must be restored to a dark adapted state before being re-exposed. Heretofore, photoconductive sheet materials have been restored to dark adapted state by heating the photoconductive sheet material at an elevated temperature or by storage in the dark for an extended period of time.

It has now been discovered that the removal of the latent image and restoration of the photoconductive material to a dark adapted state is greatly accelerated if the photoconductive sheet material is heated by placing it in contact with hot water. In this manner a photoconductive sheet can be uniformly dark adapted in the matter of a few seconds by immersion in hot water. Generally speaking, the water should be heated to at least 100° F. (preferably about 140° F.) and remain in contact with the photoconductor over a period of 10 to 60 seconds.

Photoconductor sheet materials of the type contemplated by this invention are prepared as follows:

A Waring Blender mixer is employed to thoroughly blend the following ingredients over a period of 15 minutes:

|                                                                                                            |     |
|------------------------------------------------------------------------------------------------------------|-----|
| G.                                                                                                         |     |
| Methyl-isobutyl ketone                                                                                     | 139 |
| Zinc oxide (U.S.P. 12) having a particle size of less than 40 microns                                      | 252 |
| Binder [30% toluene solution of butadiene (30 parts by weight) and styrene (70 parts by weight) copolymer] | 210 |

Sensitizing dyes are then added to the blend as 0.5% methanol solutions in order to dye-sensitize the photoconductor sheet as follows:

2

|    | Cc. |
|----|-----|
| 5  |     |
|    | 50  |
|    | 20  |
| 15 |     |
|    | 5   |
| 20 |     |
| 25 |     |
| 30 |     |
| 35 |     |
|    | 5   |
|    | 5   |

Acid Blue 1<sup>1</sup>

Br Br O O

NaO—C—Br—C—COONa

Cl Cl Cl

Acid Red 92<sup>1</sup>

N(CH<sub>3</sub>)<sub>2</sub>

C=NH<sub>2</sub>Cl<sup>+</sup>

N(CH<sub>3</sub>)<sub>2</sub>

Basic Yellow 1

<sup>1</sup> "Color Index," 2d ed., Chorley & Pickersgill Ltd., Leeds (1956)

After being blended for an additional five minutes and filtered through a coarse "sintered glass" filter, the blend was coated with a doctor blade coater onto an aluminum sheet (3 mil) to a wet thickness of .006 inch.

When dry and fully dark adapted, this sheet was used to produce reproductions and had high response spectral bands at 460—465 mu, 560 mu and 660 mu.

Because of their flexibility, durability, and resistance to crease formation, photoconductor sheet backings prepared by vapor deposition of a metal, such as aluminum, on a paper or plastic backing are especially useful. Polyethylene terephthalate films (5 mil) are preferred.

An illustrative procedure employed to prepare reproductions by the electrolytic decomposition on the surface of a zinc oxide photoconductor sheet prepared as described above and to restore the photoconductor to a dark adapted state is as follows:

(1) The negative electrode from a direct current power supply is attached to the aluminum backing of the photoconductor sheet.

(2) The photoconductor sheet retained in a developer tray is exposed uniformly to a white light source by projecting an image on the photoconductor sheet with the projector having a low F stop projection range and a 500 watt tungsten projection lamp as the light source, thereby rendering the sheet conductive. Relative hu-

midity of the atmosphere in the work area is maintained at less than 40 percent.

(3) An electrode attached to the positive terminal of the direct current power supply is placed in the developer tray.

(4) A solution of "Alcian Blue 8GN" (5 g.) which is described in "The Chemistry of Synthetic Dyes," by K. Venkataraman, Academic Press Inc., New York, N.Y. (1952), dissolved in water (100 ml.) is added to the developer tray.

(5) After a total lapse of time of about 20 seconds after exposure, a 30 volt electrical current is then passed through the photoconductor and the solution for a period of 15 seconds.

(6) The solution is removed from the developer tray 15 and the photoconductor sheet is washed with water heated to 140° F. for a period of 20 seconds to restore the photoconductor to a dark adapted state and the sheet is then dried by placing it under a stream of air. The resulting sheet had been rendered blue-green by the deposited dye.

(7) The sheet was then selectively exposed to a photographic image and titanium dioxide deposited on the exposed areas by repeating steps 3 to 5 above, using as the solution a suspension of titanium dioxide in a dilute aqueous solution of the thiuronium salt prepared by reacting N-tetradecyl-p-chloromethylbenzenesulfonamide and N,N,N',N'-tetramethyl thiourea. The titanium dioxide is deposited on the conductive areas of the photoconductor-cathode, which are areas selectively exposed to the photographic image, concurrently with the decomposition of thiuronium salt, resulting in a positive blue-green print.

We claim:

1. A process for restoring a photoconductor electrolytically developable sheet material having only latent conductivity images thereon to its dark adapted state and for washing the surface thereof which comprises contacting an organic photoconductor bonded to an electrically conductive carrier with liquid water heated to at least 100° F. and cooling the heated photoconductor to ambient temperature.

2. A process for restoring a photoconductor electrolytically developable sheet material having only latent conductivity images thereon to its dark adapted state and for washing the surface thereof which comprises contacting an organic photoconductor bonded to an electrically conductive carrier with liquid water heated to at least 100° F., drying the heated photoconductor and cooling the dry photoconductor to ambient temperature.

3. A process for restoring an electrolytically develop-

able zinc oxide photoconductor sheet material having only latent conductivity images thereon to its dark adapted state and for washing the surface thereof which comprises contacting a zinc oxide photoconductor bonded to an electrically conductive carrier liquid with water heated to at least 100° F. and cooling the heated zinc oxide to ambient temperature.

5 4. A process for restoring an electrolytically developable zinc oxide photoconductor sheet material having only latent conductivity images thereon to its dark adapted state and for washing the surface thereof which comprises contacting a zinc oxide photoconductor bonded to an electrically conductive carrier liquid with water heated to at least 100° F., drying the heated zinc oxide and cooling the dry zinc oxide to ambient temperature.

10 5. A process for dark adapting and washing a zinc oxide photoconductor sheet material which comprises contacting a zinc oxide photoconductor bonded to an electrically conductive carrier with liquid water heated to at least 100° F. and cooling the heated zinc oxide to ambient temperature, said steps being conducted under dark conditions.

20 6. A process for dark adapting and washing a zinc oxide photoconductor sheet material which comprises contacting a zinc oxide photoconductor bonded to an electrically conductive carrier with liquid water heated to at least 100° F., drying the heated zinc oxide and cooling the dry zinc oxide to ambient temperature, said steps being conducted under dark conditions.

References Cited in the file of this patent

UNITED STATES PATENTS

|              |                  |       |                |
|--------------|------------------|-------|----------------|
| 35 2,286,744 | Leatherman       | ----- | June 16, 1942  |
| 2,863,767    | Vyverberg et al. | ----- | Dec. 9, 1958   |
| 2,904,431    | Moncrieff-Yeates | ----- | Sept. 15, 1959 |
| 2,940,847    | Kaprelian        | ----- | June 14, 1960  |
| 2,987,660    | Walkup           | ----- | June 6, 1961   |
| 40 3,010,883 | Johnson et al.   | ----- | Nov. 28, 1961  |

FOREIGN PATENTS

|         |               |       |                |
|---------|---------------|-------|----------------|
| 820,763 | Great Britain | ----- | Sept. 23, 1959 |
|---------|---------------|-------|----------------|

OTHER REFERENCES

45 Perry: "Chemical Engineers' Handbook," McGraw-Hill, 1950; 3rd ed., pages 455-82 of interest.

Amick: RCA Review, December 1959, pages 753-769, 96-1PC.

Collins et al.: Physical Review, volume 112, No. 2, pages 388-395.

UNITED STATES PATENT OFFICE  
CERTIFICATE OF CORRECTION

Patent No. 3,154,414

October 27, 1964

Vsevolod Tulagin et al.

It is hereby certified that error appears in the above numbered patent requiring correction and that the said Letters Patent should read as corrected below.

Column 3, lines 34 and 35, and lines 42 and 43, for "a photoconductor electrolytically developable", each occurrence, read -- a electrolytically developable photoconductor --; same column 3, lines 38 and 46, for "organic", each occurrence, read -- inorganic --; column 4, lines 5 and 13, for "carrier liquid with", each occurrence, read -- carrier with liquid --.

Signed and sealed this 4th day of May 1965.

SEAL)

test:

RNEST W. SWIDER  
testing Officer

EDWARD J. BRENNER  
Commissioner of Patents